

May 15, 1928.

1,670,049

L. SCHERTEL ET AL

PRODUCTION OF SOLID FINELY DIVIDED MATERIAL

Filed Nov. 14, 1922



Fig. 3.  
(A--B)



Inventors:  
Siegfried Schertel  
Werner Sittig  
Oskar T. Pfeiffer

Patented May 15, 1928.

1,670,049

# UNITED STATES PATENT OFFICE.

LUDWIG SCHERTEL AND WILLI LÜTY, OF ESSEN, GERMANY, ASSIGNORS TO THE FIRM  
TH. GOLDSCHMIDT A.-G., OF ESSEN, GERMANY.

## PRODUCTION OF SOLID FINELY-DIVIDED MATERIAL.

Application filed November 14, 1922, Serial No. 600,882, and in Germany November 15, 1921.

This invention relates to the production of solid finely divided material, such as lead oxid, suitable for compositions, and various similar uses.

5 In a general aspect the invention consists in the provision of a process wherein raw material, such, for example, as molten metallic lead or pulverulent lead oxid, is distributed over and permitted to vaporize 10 from surfaces of an inert refractory material which is heated to a temperature of the order of 1000 degrees C.; and at the same time hot gases or products of combustion are permitted to flow over the surfaces thereby 15 causing the formation of a fume of lead oxid which is removed from the region of the hot surfaces and collected in a suitable manner to obtain a high yield of material in a state of extreme sub-division.

20 If molten lead be employed as the raw material the hot gases are of an oxidizing nature in order to convert the metal vapors to oxid. If lead oxid be employed as a raw material the hot gases may be products of 25 combustion. In either event a relatively large volume of gas is employed to effect the formation of a fume which is highly dispersed through the gaseous medium, and to obtain a high proportion of finely divided material with a proportionate decrease in 30 the amount of coarser particles. Coarse particles contained in the effluent mixture of gases and fume are permitted to settle out under the influence of gravity and the 35 cleaned fume is then collected or precipitated by a suitable means such as an electrical discharge.

In the accompanying drawing:

Fig. 1 is schematic longitudinal cross-40 sectional view of an apparatus for practicing our invention.

Fig. 2 is a schematic longitudinal cross-sectional view of another type of apparatus, and

45 Fig. 3 is a transverse cross-sectional view taken along the line A—B of Fig. 2.

Referring to Fig. 1, there is illustrated a tower 1 of refractory material, in which is disposed a stack of refractory bricks, 2, 50 which are slightly spaced from each other and provide a large surface area, and which are so arranged as to permit the passage of hot gases between the bricks. An inlet port 3, formed at the bottom of the tower 55 1, is provided for the admission of hot gases

from a suitable source, not shown. The upper end 1<sup>a</sup> of the tower is of somewhat larger cross-sectional area than the base thereof to effect a decrease in velocity of the gases prior to their emergence from the 60 tower. Positioned above the tower is a receptacle or hopper 4 in which is disposed a quantity 4<sup>a</sup> of raw material such as molten metallic lead or lead oxid.

The hopper 4 is provided with a port 5 opening into the tower 1 above the stack of bricks 2, which may be opened or closed by manipulating a valve 6. An exit port 7 is provided at the upper end of the tower 1, and to it is attached a pipe line 7<sup>a</sup> which 65 terminates in an electrical precipitating apparatus 8. The framework of the member 8 is connected to one pole of a generator 9, or other source of electrical energy, the other pole of which is connected to electrodes 10 disposed within the chamber 8. Under the influence of the electrical discharge, fume carried into the chamber 8 from the tower 1 is precipitated, and the conveying gases are permitted to escape 70 through a port 11. The precipitated material collects in a receptacle 12 disposed below the chamber 8 and may be removed 75 therefrom through a gate 13.

The apparatus shown in Fig. 2 comprises 85 a shell 20 having a lining of refractory material and an inlet port 21 for the admission of hot gases. A rotatable shaft 22, extending through the shell 20 is provided with a bore to permit of water cooling, and has 90 mounted thereon at intervals a plurality of perforated discs 23, consisting of, or covered with, refractory material. The shell 20 is adapted to receive a quantity of molten material 24. The discs 23 rotate within the bath 24, and carry above it thin films of raw material which is vaporized, converted to a fume by gases entering through the pipe 21, and removed to a suitable settling and precipitating apparatus through an exit 95 100 port 25.

In both types of apparatus there is provided an extensive surface area upon which the raw material may be distributed and from which it is vaporized and converted 105 to a fume.

Referring again to Fig. 1, in operation, the tower and contained brick-work 2 are brought to a suitable temperature (about 1000 C.) and molten material, such as lead,

is allowed to trickle through the port 5, fall as a spray, and distribute itself as a thin film over the brick-work. Here it is vaporized into the surrounding atmosphere and converted into a fume held in suspension by the large volume of hot gases entering through the port 3. Coarse particles of material settle out by gravity, either in the enlarged portion 1<sup>2</sup> of the tower 1, or in the pipe line 7, or both. The fume suspended in the gaseous medium is then carried forward to the chamber 8 where it is precipitated by means other than gravity. Fumes cannot be precipitated by mere gravitational action.

The resulting material, which is removed through the gate 13, is in a state of extremely fine sub-division, is uniform in quality, and has a very low apparent density. Due to the provision of a large area for effecting volatilization, excessive temperatures need not be employed, and a high yield of finished material is obtained.

It is apparent that the principles of the invention may be applied with various types of apparatus, and that the operating conditions indicated above may be varied to meet the necessities of any case. Thus, the process is applicable to the formation of finely divided antimony or tin compounds, which we regard as equivalent to plumbiferous substances. In making antimony trioxid, for example, the cylinder 20 is partially filled with molten antimony monoxid, or if desired, with molten antimony, in which case steam and products of combustion are used for heating and diluting. If antimony sulfide be employed, a limited quantity of air is used with the steam in place of products of combustion.

What we claim is:

1. The process of preparing litharge in a state of fine sub-division from simple plumbiferous material free from sulfur and halogens which comprises dispersing the raw material, distributing the same over heated refractory surfaces of large area, flowing

hot gas over the surfaces to effect the volatilization of the raw material, cooling the volatilized material and effecting the settling of particles of large size from the resultant fume and subjecting the fume to the action of a precipitating means to form a finely divided litharge.

2. The process of preparing finely divided materials from simple plumbiferous materials free from sulfur and halogens which comprises distributing the same as a film over heated refractory surfaces of large area, passing a current of gases around the surfaces, thereby effecting the volatilization of the raw material as a fume suspended in the gases, and subjecting the fume to the action of a precipitating means to separate the suspended material from the gas as a finely divided mass.

3. The process of preparing finely divided materials from metalliferous materials which comprises sub-dividing the material, passing the same through a shaft and over an extensive surface of refractory material inert with respect to the material and at a high temperature, flowing a current of hot gases over the material to effect its volatilization and to form a fume suspended in the gases, withdrawing the gaseous mass and precipitating the fume.

4. The process of preparing litharge in a state of extreme sub-division which comprises melting simple plumbiferous material free from sulfur and halogens, dispersing the same over a large area of heated refractory material, passing a counter current of hot gases over the surfaces, volatilizing the plumbiferous material, cooling the same to form a fume suspended in the gases, separating coarse particles by gravitational action, and precipitating the suspended fume from the gas to yield a finely divided litharge.

In testimony whereof, we affix our signatures.

DR. INC. LUDWIG SCHERTEL.  
DR. INC. WILLI LÜTY.